

# United States Patent Office

3,094,620

Patented June 18, 1963

1

3,094,620

## COPY-SHEET AND METHOD

John L. Reitter, St. Paul, Minn., assignor to Minnesota  
Mining and Manufacturing Company, St. Paul, Minn.,  
a corporation of Delaware  
No Drawing. Filed Jan. 3, 1961, Ser. No. 79,991  
5 Claims. (Cl. 250—65)

This invention relates to heat-sensitive copy-sheets and methods of making and using the same.

One well-known and commercially important method for copying typewritten office correspondence and other graphic originals having differentially radiation-absorptive image and background areas is known as thermographic reproduction. It involves the brief irradiation of the original, while in heat-conductive contact with a heat-sensitive copy-sheet, with high-intensity radiation. Preferential absorption of the radiation in the absorptive image areas then results in localized heating of the copy-sheet, producing a visible direct copy of the original. The background areas of the copy-sheet remain heat-sensitive.

Another commercial office copying system requires preliminary exposure of a photosensitive sheet material to actinic radiation in a pattern determined by an original having radiation-transmissive background areas. Irradiated areas are thereby rendered non-reactive. The unexposed image areas may in some instances be rendered visible by heating, but for images of effective color density the sheet must be treated with a further reagent or activator in liquid or vapor form. Apparatus for carrying out the required sequence of operations is available under the designation "Copy-Flex" Model 100 copying machine. In this apparatus the composite of copy-sheet and transparency is passed over a rotating glass cylinder containing a mercury vapor lamp. Typically, a .60 watt "UA-20B" tubular mercury lamp is located to one side of the axis of a glass cylinder having a 12 inch circumference, and the composite, in contact with the outer surface of the rotating cylinder, is exposed over an arcuate path of 6 inches at a minimum speed of one inch in 5 seconds.

Heat-sensitive copy-sheets have been described in which the visible change produced on localized brief heating is caused to occur by the inter-reaction of a metal salt and an organic chelating agent. The reaction produces a strongly colored permanent image. As previously described, however, these copy-sheets have been found to remain visibly heat-sensitive after exposure to actinic radiation at minimum speed in the Copy-Flex copying machine.

The present invention provides a heat-sensitive copy-sheet having a visibly heat-sensitive layer containing, in physically distinct and chemically inter-reactive relationship, a metal salt and an organic chelating agent capable of reacting together, in the thermographic copying process or on momentarily heating the sheet to a conversion temperature in the range of about 90° C. to about 150° C., with the formation of a visibly distinct reaction product, the reactants being rendered incapable of undergoing such reaction on exposure to actinic radiation as provided in the Copy-Flex copying machine. The invention therefore makes possible the preparation of permanent, heat-stable, high image density reproductions of graphic originals by procedures involving only irradiation and without any necessity of treatment with solutions, fumes, vapors, powders or other adjuvants.

Typically, the composite of copy-sheet and original is first briefly irradiated with intense radiation rich in infrared and in accordance with known thermographic copying procedures. The thus imaged copy-sheet is next passed through the Copy-Flex copying machine under maximum exposure to the near-ultraviolet radiation from the mer-

2

cury vapor arc. The resulting copy is stable against further heating to conversion temperature at the undarkened background areas.

Copies may alternatively be prepared by first exposing the copy-sheet to the near-ultraviolet through a transparency, for example a ribbon or carbon copy of a type-written document on thin semi-transparent paper, and then heating the entire copy-sheet to conversion temperature, for example on a heated roller or platen or in an oven.

Dithioxamide is known to be reactive with metal salts such as nickel stearate in the form of heat-sensitive copy-sheets; but such products are found to remain heat-sensitive under exposure to near-ultraviolet as just described. Surprisingly, it has now been found that substituted dithioxamide such as N,N'-bis furfuryl dithioxamide are equally effectively reactive with nickel stearate in copy-sheet formulations at conversion temperatures, while at the same time making possible the complete desensitization of the copy-sheet against such reaction by a single pass through the Copy-Flex machine.

The substituted dithioxamide and metal salt may be intimately dispersed in a thin film of a resinous or polymeric film-forming binder, either in self-sustaining film form or as a coating on a paper, film or other paper-like backing, providing a unitary heat-sensitive copy-sheet in a single coating and drying operation. The two reactants may separately be dispersed or dissolved together with appropriate binders, and applied to a paper-like backing in separate coatings with intermediate drying, or to separate backings. In the latter case the two sheets when held in face-to-face contact permit interfacial reaction at conversion temperature. The relative amounts of the two reactants are not critical, particularly in structures wherein the image-forming reaction occurs at an interface, the only requirement being that sufficient of each reactant be present to ensure a readily visible change on reaction. It is desirable to employ a minimum amount of the substituted dithioxamide and to maintain this material in position for maximum exposure to the actinic radiation.

Various additives are useful in providing copy-sheets of improved appearance, handling characteristics, or other properties. Pigments, fillers, plasticizers, dyes, waxes, resins and other additives may be incorporated.

The following specific examples will further illustrate but not limit the invention. Proportions are given in parts by weight.

### EXAMPLE 1

| Mixture A               |      |
|-------------------------|------|
| Nickel stearate         | 6.6  |
| Silica powder           | 2.3  |
| Polyvinyl acetate resin | 4.6  |
| Acetone                 | 86.5 |

### Mixture B

|                                |      |
|--------------------------------|------|
| N,N'-bis furfuryl dithioxamide | 0.1  |
| Ethyl cellulose                | 5.0  |
| Acetone                        | 94.9 |

Mixture A is prepared by prolonged milling in a ball mill, and is then coated in a thin uniform layer on map overlay tracing paper and dried. Mixture B is prepared by mixing the components together until solution is effected. The solution is then applied as a thin uniform coating over the previous coating and the sheet is again dried. There is obtained a heat-sensitive copy-sheet having a neutral color. Local heating, as by momentary contact of the sheet with a metal test bar at 150° C., causes intense darkening.

A portion of the copy-sheet is placed beneath a graphic

original prepared by typing on thin paper and the composite is irradiated in accordance with thermographic copying procedure. A sharp and clear reproduction of the typed characters is obtained. The copy is then exposed for approximately 30 seconds to intense near-ultraviolet radiation by passing it through the Copy-Flex copying machine at minimum speed. The dark image areas remain unchanged. The background areas no longer darken when placed in momentary contact with the heated test bar.

A separate portion of the copy-sheet is placed beneath a printed transparency prepared by typing on thin semi-transparent paper, and the composite is exposed to near-ultraviolet radiation by passing it through the Copy-Flex copying machine as before. With the copy-sheet and transparency maintained in register, the composite is next briefly irradiated as for thermographic copying. The resulting copy has sharply defined dark image areas on a neutral background and is stable against further heating at 150° C.

The image areas are equally readily developed by replacing the transparency with a sheet of radiation-absorbent black paper prior to irradiating the composite with infra-red, or by placing the copy-sheet in contact with a heated metal platen or roller or in an oven heated to about 150° C.

With N,N'-bis furfuryl dithiooxamide and nickel stearate as the reactant materials, a purple image color is obtained. Nickel stearate with N,N'-bis carboxyamyl dithiooxamide provides a pink image. Other salts of nickel, such for example as nickel behenate, produce similar results. Salts of cobalt and copper are also useful. Other non-inventive variations will be apparent in view of the foregoing disclosures.

The compound N,N'-bis(furfuryl)dithiooxamide having the structural formula



is prepared by condensation of dithiooxamide with two mols of furfurylamine in accordance with the procedure described in the pamphlet entitled "Dithiooxamide and Its N,N'-Disubstituted Derivatives" and copyrighted in 1959 by Mallinkrodt Chemical Works. The compound N,N'-biscarboxyamyl dithiooxamide, having the formula



is similarly prepared using dithiooxamide and amino-caproic acid.

What is claimed is as follows:

1. A heat-sensitive copy-sheet capable of undergoing permanent visible change on being momentarily heated to a conversion temperature within the range of about 90° C. to about 150° C. and of becoming insensitive to said heating on moderate exposure to near-ultraviolet radiation, said copy-sheet including a visibly heat-sensi-

tive layer containing, in physically distinct and chemically inter-reactive relationship, chemically inter-reactant consisting essentially of nickel stearate and N,N'-bis furfuryl dithiooxamide.

5 2. A unitary heat-sensitive copy-sheet capable of undergoing permanent visible change on being momentarily heated to a conversion temperature within the range of about 90° C. to about 150° C. and of becoming insensitive to said heating on moderate exposure to near-ultraviolet radiation, said copy-sheet comprising a thin paper-like backing and a coating comprising a film-forming binder and, in physically distinct and chemically inter-reactive relationship, chemically inter-reactant components consisting essentially of nickel stearate and N,N'-bis furfuryl dithiooxamide.

10 3. Method of copying comprising placing in surface contact and in position for irradiation a graphic original having differentially infra-red-absorptive image and background areas and a heat-sensitive copy-sheet having a visibly heat-sensitive layer containing nickel stearate and N,N'-bis furfuryl dithiooxamide in physically distinct and chemically inter-reactive relationship, momentarily irradiating said graphic original with intense radiation rich in infra-red for causing visible inter-reaction in said layer at image-defining areas, and then irradiating said layer with radiation in the near-ultraviolet range for rendering the background areas visibly insensitive to subsequent heating.

15 4. Method of copying comprising subjecting a heat-sensitive copy-sheet, having a visibly heat-sensitive layer containing nickel stearate and N,N'-bis furfuryl dithiooxamide in physically distinct and chemically inter-reactive relationship, to an exposure to intense radiation in the near-ultraviolet wavelength region and in localized background-defining areas sufficient to render said areas selectively insensitive to heat, and then heating at least the image-defining areas of said layer to provide a visible image.

20 5. A radiation-desensitizable intermediate sheet product suitable for use in the reproduction of a graphic original by a process involving heating said sheet product, while in face-to-face contact with a separate receptor sheet consisting essentially of a paper-like backing and a surface layer of nickel stearate, at areas corresponding to image-forming areas of said original; the said intermediate sheet product consisting essentially of a paper-like backing and a surface layer of N,N'-bis-furfuryl dithiooxamide.

25 50 References Cited in the file of this patent

UNITED STATES PATENTS

|           |               |                |
|-----------|---------------|----------------|
| 2,482,815 | Urbach        | Sept. 27, 1949 |
| 2,813,042 | Gordon et al. | Nov. 12, 1957  |
| 2,910,377 | Owen          | Oct. 27, 1959  |
| 2,936,276 | Chalkley      | May 10, 1960   |
| 2,950,987 | Howard        | Aug. 30, 1960  |
| 2,967,785 | Allen et al.  | Jan. 10, 1961  |